

# UNITED STATES PATENT OFFICE.

HUGH S. COOPER, OF CLEVELAND, OHIO, ASSIGNOR TO THE COOPER RESEARCH COMPANY, OF CLEVELAND, OHIO, A CORPORATION.

## ALLOY.

1,254,987.

Specification of Letters Patent. Patented Jan. 29, 1918.

No Drawing.

Application filed October 15, 1917. Serial No. 196,592.

*To all whom it may concern:*

Be it known that I, HUGH S. COOPER, citizen of the United States, residing at Cleveland, in the county of Cuyahoga and State of Ohio, have invented certain new and useful Improvements in Alloys, of which the following is a specification.

This invention relates to an improved alloy, comprising aluminum and beryllium, and my object is to combine these metals in suitable proportions to provide an alloy of superior properties and characteristics compared with other light-weight metal alloys in use or known at the present time.

In the periodic table, beryllium is classed with several other metals, among which are the light metals magnesium and calcium. In appearance it is of a silvery color, and is permanent in air. It is very ductile and malleable, and the melting point which is about 1500° C. is very high for a metal of this class. It is slightly heavier than magnesium with a specific gravity of about 1.80. It is not affected by water, either hot or cold, and is much harder than aluminum, calcium or magnesium.

The most common mineral containing this metal is beryl which contains about twelve per cent. of the oxid and is a silicate of this metal with aluminum. This mineral is quite widely distributed throughout the world and is found in large amounts in the Eastern States of this country where it occurs in massive crystals of several hundred pounds in weight.

To obtain alloys of this metal with aluminum at a relatively low cost commercially, one procedure is to subject to the action of an electric current a bath containing the mixed oxides of aluminum and beryllium, which are held in solution, said bath being of course a conducting medium, and in this manner obtain an alloy of the two metals at a much lower cost than if salts of these two metals were first separated by chemical means, the metals then extracted and melted together to make the alloys.

Where the method employed in the extraction of beryllium is expensive, I prefer to make the alloy of preponderating amounts of aluminum and lesser amounts of beryllium, using such relatively small amounts

of beryllium as will impart to aluminum sufficient valuable properties as to justify the production of this alloy on a commercial scale. Where the method permits the production of beryllium at a low cost, an alloy made of a preponderating amount of beryllium is preferred, such alloy being much lighter in weight for one thing than an alloy having a lower percentage of beryllium.

An alloy prepared by melting together the two metals named is much stronger than aluminum, alone; it is harder and possesses a higher melting point than aluminum alone, and is from five per cent. to thirty per cent., lighter, depending upon the amount of beryllium contained.

Such an alloy is permanent in water, either boiling or cold; retains a polish for a considerable period; is very easy to machine, and makes very excellent castings. Within certain limits the alloy is ductile and malleable, and may be drawn, rolled or pressed into various products.

I have found that small amounts of this element, say from one to five per cent., combined with aluminum, greatly increases the tensile strength of aluminum, even beyond that obtained with magnesium; and by increasing these amounts it is possible to retain this strength and at the same time produce alloys variably lighter than aluminum, depending upon the amount of beryllium contained.

Under a high cost of beryllium, it is advisable to use from one per cent. to about twenty per cent., beryllium, with the balance aluminum. However, alloys with preponderating amounts of beryllium, say from sixty-five per cent. to about ninety-nine per cent. will prove even more valuable commercially where the cost is reduced, being much lighter than the former alloys and from twenty per cent. to thirty per cent. lighter than aluminum.

What I claim is:

1. An alloy composed of the metals aluminum and beryllium.
2. An alloy, comprising aluminum and one per cent. to ninety-nine per cent. beryllium.
3. An alloy, comprising beryllium and a metal in the class embracing aluminum.

4. An alloy possessing greater strength and less weight than aluminum, comprising aluminum and beryllium, the aluminum being in preponderating amount.
5. An alloy which is stronger, harder and of lighter weight than aluminum, consisting of aluminum and less than sixty-five per cent. beryllium.
6. An alloy, composed of one to twenty per cent. beryllium, with the balance aluminum.

Signed at Cleveland, in the county of Cuyahoga and State of Ohio, this 10th day of October, 1917.

HUGH S. COOPER.